# EUROPEAN PATENT SPECIFICATION

(11) **EP 3 238 791 B1**
(45) Date of publication and mention of the grant of the patent: **15.01.2020**
(21) Application number: 17168228.9
(22) Date of filing: 26.04.2017
(51) Int. Cl.: A63C 5/04, A63C 5/044

(54) **METHOD FOR TREATING A SLIDING SURFACE OF A SLIDING DEVICE AND THE SLIDING DEVICE COMPRISING THAT SLIDING SURFACE**
METHODE ZUR BEHANDLUNG EINER GLEITFLÄCHE EINES GLEITGERÄTS UND DAS GLEITGERÄT MIT DIESER GLEITFLÄCHE
MÉTODE DE TRAITEMENT UNE SEMMELLE DE GLISSE D'UN APPAREIL DE GLISSE ET L'APPAREIL DE GLISSE COMPRENANT CETTE SEMELLE

(30) Priority: 26.04.2016 IT UA20162890
(43) Date of publication of application: 01.11.2017
(73) Proprietor: PENZ S.R.L., 23823 Colico (LC) (IT); Politecnico di Milano, 20133 Milano (IT)
(72) Inventor: Ripamonti, Francesco, 22036 Erba (CO) (IT); Ossi, Paolo Maria, 19015 Levanto (SP) (IT); Moro, Mario Francesco, 23020 Piuro (SO) (IT)
(74) Representative: Petraz, Gilberto Luigi

(56) References cited:
- EP-A1- 0 785 000
- EP-A1- 1 415 686
- WO-A1-03/000483
- DE-A1-102005 026 097
- JP-A- H09 300 002
- US-A1- 2006 251 486

## Description

### FIELD OF THE INVENTION

The present invention concerns a method for treating a base for sliding apparatuses, for example skis or suchlike, used in winter sports for sliding on snow-covered ground or suchlike, including ground prepared with artificial snow and similar materials, which have high sliding properties. The present invention also concerns a base for a sliding apparatus and the sliding apparatus itself, used in particular for winter sports.

In the case of a pair of skis, by the term "sliding apparatus" we mean, hereafter in the description, each of the skis used for sliding or gliding on snow-covered ground or suchlike.

### BACKGROUND OF THE INVENTION

It is known that modern sliding apparatuses used in particular in winter sports consist of a structure provided with layers of different materials overlapping on each other.

On a macroscopic level, the multi-layer structure that the sliding structure is made of is similar in most types of modern sliding apparatuses present on the market. However, the individual layers can be made with different geometries and materials or a different composition of materials, in order to obtain the desired characteristics, for example in terms of flexibility and manageability of the apparatus. The techniques for assembling and producing normal sliding apparatuses are also consolidated and used by most producers.

From a functional point of view, and especially in the practice of Alpine and Nordic skiing, the sliding properties of the sliding apparatus are a fundamental feature for performance, both in competitive sport and also in terms of the manageability and usability of the apparatus.

Therefore, the study of slidability and of the parameters that influence the dynamic sliding friction between the sliding apparatus and the snow-covered ground, and therefore, in short, between the base of the sliding apparatus and the snow-covered ground, is extremely important.

The tribology of the base of the sliding apparatus can be influenced by various parameters, including, principally, the characteristics of the material or materials it is made of, the sliding surface and the treatment of the base able in general to reduce to a minimum the dynamic friction between base and snow.

In order to improve the sliding characteristics of such sliding apparatuses on the snow, it is known, as mentioned above, to use various types of material and various surface working techniques, especially for the bases. However, known materials and working techniques for ski apparatuses do not allow to obtain ski apparatuses provided with optimum slidability and characteristics that allow optimum control during normal prolonged use, possibly for different morphologies of the snow cover.

EP 1 415 686 A1 discloses a process and apparatus for structuring the running sole of a snow sliding board like a ski or a snowboard, and corresponding sliding apparatus. A roller is pressed against the running surface which is fitted with peripheral and free-rotating bodies, in a ball cage, which embosses the surface material. The embossed surface is smoothed so that the displaced material from the embossed recesses is forced back into the running surface. The sole shows a plurality of craters (recesses) and ridges (displaced material), but no working step or working process is carried out inside the craters. Moreover the dimensions of the recesses and of the ridges obtained by the displaced material are not specified.

US 2006/251486 A1 describes a method for machining the running surfaces of winter sports appliances such as skis or snowboards, in which a blank track is subjected to a machining process in order to obtain a predetermined surface microstructure, which improves the gliding ability. A precisely defined and reproducible surface structure of the track is achieved in such a way that the machining process for producing the surface microstructure comprises a plastic deformation by a tool which is moved over a running surface of the track blank and is pressed with a predetermined force on the track blank in order to deform the same in a plastic manner. It does not describe any working step or working process carried out inside the depressions delimited by two elevations obtained by means of the tool. The vertical dimension of the depression is approximately 0.015 mm. The vertical dimension of the elevation is approximately 0.01 mm. The total height is thus approximately 0.025 mm.

Furthermore, known ski apparatuses can have various problems regarding the wear of the materials, and therefore it often needs different and costly maintenance operations, both for the base and also the edges.

Other limitations and disadvantages of conventional solutions and technologies will be clear to a person of skill after reading the remaining part of the present description with reference to the drawings and the description of the embodiments that follow.

There is therefore a need to perfect a method for treating a base of a sliding apparatus and to obtain a base suitable for a sliding apparatus which can overcome at least one of the disadvantages of the state of the art.

One purpose of the present invention is therefore to perfect an effective and precise method for treating a base for a sliding apparatus, in particular a sliding apparatus for sliding on snow-covered terrains, by means of which the base obtained has optimum sliding qualities on the snow and therefore by means of which the dynamic friction between the sliding apparatus in which it is installed and the snow-covered ground is reduced to a minimum.

Another purpose of the present invention is to perfect a method for treating a base for a sliding apparatus, in particular a sliding apparatus for sliding on snow-covered terrains, which allows to obtain a base and therefore in general a sliding apparatus which is durable and therefore in which the wear deriving from normal use is significantly reduced and which also requires minimum interventions in terms of maintenance compared with known bases and sliding apparatuses.

Another purpose of the present invention is to obtain a base for a sliding apparatus, in particular a sliding apparatus for snow-covered ground, which in its entirety is more efficient and performs better (greater precision in trajectories) compared with normal bases for sliding apparatuses known in the field.

Another purpose of the present invention is to obtain a sliding apparatus which is in its entirety is more efficient and long-lasting, and performs better in terms for example of precision in trajectories compared with known apparatuses.

The Applicant has devised, tested and embodied the present invention to overcome the shortcomings of the state of the art and to obtain these and other purposes and advantages.

### SUMMARY OF THE INVENTION

The present invention is set forth and characterized in the independent claims, while the dependent claims describe other characteristics of the invention or variants to the main inventive idea.

The subject-matter of the present invention is defined in independent claims 1, 7 and 10.

In accordance with the above purposes and according to a first aspect of the invention, a method for treating a base able to be used in a sliding apparatus and provided with at least a sliding surface, comprises at least a first step of cutting the base by means of which a plurality of craters with a controlled depth and diameter are made on the sliding surface, and at least a second step of structuring and finishing the sliding surface in zones of the sliding surface defined inside the craters and in zones of the sliding surface defined between one crater and the other, so as to obtain a plurality of ridges distributed on the sliding surface of the base in the craters and between one crater and the other. The craters have micrometric sizes and the ridges have nanometric sizes.

Preferably, at the end of the first cutting step, the craters are distributed in a preferably regular pattern on the sliding surface of the base.

According to another aspect of the invention, the first cutting step is performed using a pulsed laser and allows to obtain craters of micrometric sizes.

Preferably, the craters have a depth variable between about 0.5 µm and about 50 µm.

Preferably, the craters have a diameter variable between about 5 µm and about 100 µm and preferably less than 50 µm.

The procedure for finishing and structuring the sliding surface is a nanostructuring procedure performed by an ionic erosion process on the sliding surface.

The invention also concerns a sliding base comprising at least a sliding surface. A plurality of craters are made in the sliding surface having micrometric sizes, a controlled depth and diameter and a plurality of ridges having nanometric sizes and in zones of the sliding surface of the base inside the craters and in zones situated between one crater and the other.

Preferably, the base is made by at least one layer of metal material or metal alloys.

The base can have a thickness variable between about 0.2 mm and about 0.8 mm.

The invention also concerns a sliding apparatus comprising a plurality of overlapping layers and at least one base provided with at least one sliding surface. The sliding surface comprises a plurality of craters having micrometric sizes and having a controlled depth and diameter and a plurality of ridges having nanometric sizes and distributed in zones of the sliding surface of the base inside the craters and in zones situated between one crater and the other.

Preferably the sliding apparatus comprises edges made in a single piece with the base.

These and other aspects, characteristics and advantages of the present disclosure will be better understood with reference to the following description, drawings and attached claims. The drawings, which are integrated and form part of the present description, show some forms of embodiment of the present invention, and together with the description, are intended to describe the principles of the disclosure.

The various aspects and characteristics described in the present description can be applied individually where possible. These individual aspects, for example aspects and characteristics described in the attached dependent claims, can be the object of divisional applications.

It is understood that any aspect or characteristic that is discovered, during the patenting process, to be already known, shall not be claimed and shall be the object of a disclaimer.

### BRIEF DESCRIPTION OF THE DRAWINGS

These and other characteristics of the present invention will become apparent from the following description of some embodiments, given as a non-restrictive example with reference to the attached drawings wherein:
- fig. 1 is a partial front view and in cross section of a sliding apparatus comprising a sliding base according to the present invention;
- fig. 2 is a schematic view from below of the base of the sliding apparatus;
- fig. 3 is a view on a larger scale compared to fig. 2 and relating to a zone of the surface of the base treated according to the present method;
- fig. 4 is a view on a larger scale compared to fig. 3 and relating to a group of craters made on the sliding surface of the base;
- fig. 5 is a schematic view in lateral elevation of a crater, in particular a micro crater, made on the sliding surface of the base;
- fig. 6 is a first image taken using an electronic scan microscope of one of the craters made on the sliding surface of the base at the end of working with pulsed laser (LST, Laser Surface Texturing);
- fig. 7 is a second image taken using an electronic scan microscope of the crater in fig. 5 at the end of another working using ionic erosion of the sliding surface of the base.

To facilitate comprehension, the same reference numbers have been used, where possible, to identify identical common elements in the drawings. It is understood that elements and characteristics of one embodiment can conveniently be incorporated into other embodiments without further clarifications.

### DETAILED DESCRIPTION OF SOME EMBODIMENTS

We shall now refer in detail to the various embodiments of the present invention, of which one or more examples are shown in the attached drawings. Each example is supplied by way of illustration of the invention and shall not be understood as a limitation thereof. For example, the characteristics shown or described insomuch as they are part of one embodiment can be adopted on, or in association with, other embodiments to produce another embodiment. It is understood that the present invention shall include all such modifications and variants.

Before describing these embodiments, we must also clarify that the present description is not limited in its application to details of the construction and disposition of the components as described in the following description using the attached drawings. The present description can provide other embodiments and can be obtained or executed in various other ways. We must also clarify that the phraseology and terminology used here is for the purposes of description only, and cannot be considered as limitative.

With reference to the attached drawings, a sliding apparatus 10 comprises a structure in which can be distinguished, starting from the bottom, a series of overlapping layers of the desired thickness, that is to say: a sliding base 11; a layer 12 of glass fiber or carbon fiber located above the base 11 and made for example of cross-laminated glass; a layer 13 of glass fiber or carbon fiber located above layer 12, for example a layer of cross-laminated glass; a layer 14 with anti-vibration functions, made for example of rubber or suchlike; a central core 15, made for example of multi-layer wood; a layer 16 of glass fiber or carbon fiber, located above the central core 15 and made for example of unidirectional laminate; a layer 17 of glass fiber or carbon fiber located above layer 16 and made for example of cross-laminated glass; another layer 18 with anti-vibration functions, made of rubber or suchlike for example; and an upper layer 19, preferably made of plastic material, for example with a base of thermoplastic polymers.

On each side of the sliding apparatus 10 a sidewall 20 is also positioned, made for example of thermoplastic material, such as acrylonitrile-butadiene-styrene (ABS) or suchlike.

In the solution proposed according to the present invention, the base 11 of the sliding apparatus 10, which comprises a sliding surface 21 preferably made of metal material, integrates in a single piece the edges normally provided in any sliding apparatus and is produced starting from a strip with a thickness comprised between 0.2 and 0.8 mm for example, which therefore represents the thickness of the base 11.

By way of example, as materials for the basic strip from which the base 11 is obtained with standard cutting methods, it is possible to use different types of metal materials, for example a first alloy with the commercial name of Titanal®, which is substantially an aluminum alloy, or stainless steel INOX AISI 301, which gives a better mechanical performance, or other metal materials, also combined with each other.

To produce the base 11 of the sliding apparatus according to the invention, the strip is cut and shaped using a method similar to that used for conventional bases made of polymer such as UHMWPE (Ultra High Molecular Weight Polyethylene), then integrated into the sliding apparatus 10 using operations such as for example hot gluing and pressing.

At the end of these operations there follows a surface finishing step on the base 11, carried out with a level of precision such as to guarantee optimum efficiency and performance.

After the surface finishing step, a hierarchical structuring is prepared, which provides for example a nano and microscopic control of the surface of the base 11. The hierarchical structuring step is preferably divided into two working steps.

In the first step, a cutting process is made on the sliding surface 21, for example with a pulsed laser (Laser Surface Texturing, LST), using a known machine and suitable for the purpose, for example equipped with a nanosecond laser, which currently represents a good compromise between efficiency and total working costs.

As a result, on the sliding surface 21 of the base 11 a sequence of craters 22 is produced, therefore obtained by laser irradiation.

In this first working step another type of laser could also be used, for example a femtosecond ultrafast laser.

Alternatively, the craters 22 obtained at the end of the first cutting step could be made using different techniques, for example by rollers provided with suitably sized indentations.

Each of the craters 22 will have a predetermined and controlled depth P and diameter D, so as to optimize the sliding performance and durability of the base 11 and hence of the sliding apparatus 10 in its entirety.

It has been found that a depth P of the craters 22 which confers particular characteristics of slidability and efficiency on the base 11 applicable to the sliding apparatus 10 varies from about 0.5 µm to about 50 µm.

It has been found that a diameter D of the craters 22 which confers particular characteristics of slidability and efficiency on the base 11 applicable to the sliding apparatus 10 varies from about 5 µm and about 100 µm and is preferably less than 50 µm.

In any case, these values of the depth P and diameter D of the craters 22 can be modified according to the technical characteristics and the type of sliding apparatus 10 to be obtained, depending for example whether it is used for Alpine skiing, cross country or other disciplines. Moreover, the parameters must also take into account the conditions of morphological variability of the snow cover.

After this first working step (see also figs. 3 and 4), the sliding surface 21 is covered by craters 22 disposed preferably in an orderly manner and a regular pattern 23, so as to guarantee a uniform treatment of the sliding surface 21 of the base 11.

In this case, by way of example, we have shown a regular pattern 23 formed by craters 22 aligned in lines and columns but naturally this regular pattern 23 could be made with different distributions, for example irregular distributions.

In fig. 2 the craters 22 distributed in a regular pattern 23 are shown only in a circled zone of the sliding surface 21 of the base 11; however, preferably, the regular pattern 23 of craters 22 will be made uniformly over the whole sliding surface 21 of the base 11.

At the end of the first laser working step, it may be provided to smooth the base 11, to remove the flashes associated with the first working step.

At this point, once the craters 22 have been made with suitable depth P and diameter D on the sliding surface 21 of the base 11, the second step of finishing and structuring is begun, comprising a nanostructuring of the sliding surface 21.

The operation to nanostructure the sliding surface 21 takes place both in zones of the sliding surface 21 comprised inside the craters 22, and also in zones of the sliding surface 21 outside the craters 22, that is, defined between one crater and the other.

The purpose of this process is substantially to make a series of ridges 24, preferably of nanometric size, which are disposed inside and around each crater 22, uniformly, as shown schematically in fig. 4 and as shown by the image in fig. 6.

The finishing and nanostructuring operation can be performed by an ionic erosion process, where the target consists of the base 11 and in particular its sliding surface 21.

As is known, in ionic erosion processes, the target is inserted in an environment where a vacuum has been created and it is subjected to a bombardment of ions, for example argon ions, so that the surface atoms of the material it consists of, in this case the sliding surface 21, are expelled. In short the ridges 24 with nanometric sizes are obtained on the sliding surface 21.

The ionic erosion process can be performed by passive devices able to generate magnetic fields, by means of radiofrequency, or by maintaining a continuous current inside the vacuum environment where the target is positioned, hence the base 11 with its sliding surface 21.

For example, in the case of radiofrequency ionic erosion, the values of radiofrequency can be 13.56 MHz, as per international standards.

The pressure of the atmosphere inside the environment where the target is positioned, i.e. the sliding surface 21 of the base 11, is controlled in the range of tens of Pa, if necessary, starting from a reference vacuum in the range of 10⁻⁴ Pa.

The ionic erosion power varies according to the metal or metal alloy that the base 11 is made of, and can vary for example between 50 W and 125 W.

The nanostructuring process through ionic erosion can be carried out in a plurality of different steps, separated by pauses. Indeed it has been found that dividing the ionic erosion process into different steps allows to obtain a better nanostructuring of the sliding surface 21.

There can be, for example, three ionic erosion steps and each of them can have a predetermined duration of about 10 minutes. The intervals between one ionic erosion step and the next can also have a duration of about 10 minutes.

As a result therefore, a base 11 is obtained which is preferably treated with the operations as described above over the whole width of the sliding surface 21. As we said, advantageously, the sliding apparatus 10 on which the base 11 will be mounted will have the edges made in a single piece, that is, integrated with the base 11.

Experiments have been carried out to compare the solution with a known base made of polyethylene and the solution according to the present invention, made for example of Titanal® or stainless steel INOX AISI 301.

The experiments were conducted making a rectilinear descent on a course with an almost constant slope. The environmental conditions were normal (T = -1°C, RU = 73%). Two indexes were monitored:
- initial acceleration, strictly correlated to the friction of first departure;
- travel time, strictly correlated to the mean value of dynamic friction during the test.

The following Table shows the mean values (the tests were repeated several times) compared with the known solution of polyethylene base.

As can be seen, the base according to the present invention, both when made of Titanal® and when made of INOX AISI 301, has irrefutable advantages both in terms of initial acceleration and in terms of travel compared with known bases made of polyethylene.

| **Solution** | **Initial acceleration** | **Travel time** |
|---|---|---|
| Titanal® vs polyethylene | +15.9% | -7.1% |
| AISI301 vs polyethylene | +14.8% | -5.1% |

It is clear that modifications and/or additions of parts may be made to the method for treating a sliding apparatus and the sliding apparatus as described heretofore, without departing from the field and scope of the present invention.

It is also clear that, although the present invention has been described with reference to some specific examples, a person of skill in the art shall certainly be able to achieve many other equivalent forms of method for treating a sliding apparatus and the sliding apparatus itself, having the characteristics as set forth in the claims and hence all coming within the field of protection defined thereby.

In the following claims, the sole purpose of the references in brackets is to facilitate reading: they must not be considered as restrictive factors with regard to the field of protection claimed in the specific claims.

## Claims

1. Method for treating a base (11) able to be used in a sliding apparatus (10) and provided with at least a sliding surface (21), comprising at least a first step of cutting the base (11) by means of which a plurality of craters (22) are made on the sliding surface (21), said craters (22) having micrometric sizes and having a controlled depth (P) and diameter (D), and at least a second step of structuring and finishing said sliding surface (21) in zones of said sliding surface (21) defined inside the craters (22) and in zones of said sliding surface (21) defined between one crater (22) and the other, so as to obtain a plurality of ridges (24) having nanometric sizes and distributed on the sliding surface (21) of the base (11), in said craters (22) and between one crater (22) and the other.

2. Method as in claim 1, **characterized in that** at the end of said first cutting step said craters (22) are distributed in a preferably regular pattern (23) on the sliding surface (21) of the base (11).

3. Method as in any claim hereinbefore, **characterized in that** said first cutting step is performed using a pulsed laser.

4. Method as in any claim hereinbefore, **characterized in that** said craters (22) have a depth (P) variable between about 0.5 µm and about 50 µm.

5. Method as in any claim hereinbefore, **characterized in that** said craters (22) have a diameter (D) variable between about 5 µm and about 100 µm and preferably less than 50 µm.

6. Method as in any claim hereinbefore, **characterized in that** said finishing and structuring procedure on the sliding surface (21) is a nanostructuring procedure performed by an ionic erosion process on the sliding surface (21).

7. Sliding base comprising at least a sliding surface (21), wherein said sliding surface (21) comprises a plurality of craters (22) having micrometric sizes and having a controlled depth (P) and diameter (D) and a plurality of ridges (24) having nanometric sizes and distributed in zones of the sliding surface (21) of the base (11) inside said craters (22) and in zones situated between one crater (22) and the other.

8. Base as in claim 7, **characterized in that** said base (11) is made by at least one layer of metal material or metal alloys.

9. Base as in claim 7 or 8, **characterized in that** said base (11) has a thickness variable between about 0.2 mm and about 0.8 mm.

10. Sliding apparatus comprising a plurality of overlapping layers (12-19) and at least one base (11) provided with at least one sliding surface (21), wherein said sliding surface (21) comprises a plurality of craters (22) having micrometric sizes and having a controlled depth (P) and diameter (D) and a plurality of ridges (24) having nanometric sizes and distributed in zones of the sliding surface (21) of the base (11) inside said craters (22) and in zones situated between one crater (22) and the other.

11. Sliding apparatus as in claim 10, **characterized in that** it comprises edges made in a single piece with the base (11).

## Patentansprüche

1. Verfahren zur Behandlung einer Basis (11), die geeignet ist, in einem Gleitgerät (10) verwendet zu werden und mit mindestens einer Gleitfläche (21) ausgestattet ist, umfassend mindestens einen ersten Schritt des Einschneidens der Basis (11), wodurch eine Vielzahl an Kratern (22) auf der Gleitfläche (21) ausgebildet wird, wobei die Krater (22) mikrometrische Größen aufweisen und eine festgelegte Tiefe (P) und einen festgelegten Durchmesser (D) aufweisen, und mindestens einen zweiten Schritt der Strukturierung und der Endbearbeitung der Gleitfläche (21) in Bereichen der Gleitfläche (21), die innerhalb der Krater (22) definiert werden, und in Bereichen der Gleitfläche (21), die zwischen einem Krater (22) und dem anderen definiert werden, so dass eine Vielzahl an Graten (24), welche nanometrische Größen aufweisen und auf der Gleitfläche (21) der Basis (11) verteilt sind, in den Kratern (22) und zwischen einem Krater (22) und dem anderen erhalten wird.

2. Verfahren gemäß Anspruch 1, **dadurch gekennzeichnet, dass** am Ende des ersten Einschneideschritts die Krater (22) in einem vorzugsweise gleichmäßigen Muster (23) auf der Gleitfläche (21) der Basis (11) verteilt sind.

3. Verfahren gemäß irgendeinem der vorhergehenden Ansprüche, **dadurch gekennzeichnet, dass** der erste Einschneideschritt unter Verwendung eines gepulsten Lasers durchgeführt wird.

4. Verfahren gemäß irgendeinem der vorhergehenden Ansprüche, **dadurch gekennzeichnet, dass** die Krater (22) eine variable Tiefe (P) zwischen etwa 0,5 µm und etwa 50 µm aufweisen.

5. Verfahren gemäß irgendeinem der vorhergehenden Ansprüche, **dadurch gekennzeichnet, dass** die Krater (22) einen variablen Durchmesser (D) zwischen etwa 5 µm und etwa 100 µm und vorzugsweise von weniger als 50 µm aufweisen.

6. Verfahren gemäß irgendeinem der vorhergehenden Ansprüche, **dadurch gekennzeichnet, dass** das Endbearbeitungs- und Strukturierungsverfahren auf der Gleitfläche (21) ein Nanostrukturierungsverfahren ist, das durch einen ionischen Erosionsprozess auf der Gleitfläche (21) durchgeführt wird.

7. Gleitbasis umfassend mindestens eine Gleitfläche (21), wobei die Gleitfläche (21) eine Vielzahl an Kratern (22) umfasst, welche mikrometrische Größen aufweisen und festgelegte Tiefen (P) und Durchmesser (D) aufweisen, und eine Vielzahl an Graten (24) umfasst, welche nanometrische Größen aufweisen und in Bereichen der Gleitfläche (21) der Basis (11) innerhalb der Krater (22) und in Zonen, die zwischen einem Krater (22) und dem anderen gelegen sind, verteilt sind.

8. Basis gemäß Anspruch 7, **dadurch gekennzeichnet, dass** die Basis (11) aus mindestens einer Schicht eines Metallmaterials oder Metalllegierungen gefertigt ist.

9. Basis gemäß Anspruch 7 oder 8, **dadurch gekennzeichnet, dass** die Basis (11) eine Dicke zwischen etwa 0,2 mm und etwa 0,8 mm aufweist.

10. Gleitgerät umfassend eine Vielzahl an sich überlagernden Schichten (12-19) und mindestens eine Basis (11), die mit mindestens einer Gleitfläche (21) ausgestattet ist, wobei die Gleitfläche (21) eine Vielzahl an Kratern (22) umfasst, welche mikrometrische Größen aufweisen und festgelegte Tiefen (P) und Durchmesser (D) aufweisen, und eine Vielzahl an Graten (24) umfasst, welche nanometrische Größen aufweisen und in Bereichen der Gleitfläche (21) der Basis (11) innerhalb der Krater (22) und in Zonen, die zwischen einem Krater (22) und dem anderen gelegen sind, verteilt sind.

11. Gleitgerät gemäß Anspruch 10, **dadurch gekennzeichnet, dass** es Kanten umfasst, die in einem Stück mit der Basis (11) gefertigt sind.

## Revendications

1. Procédé de traitement d'une base (11) apte à être utilisée dans un appareil de glissement (10) et munie d'au moins une surface de glissement (21), comprenant au moins une première étape de coupe de la base (11) au moyen de laquelle une pluralité de cratères (22) sont réalisés sur la surface de glissement (21), lesdits cratères (22) ayant des dimensions micrométriques et ayant une profondeur (P) et un diamètre (D) contrôlés, et au moins une deuxième étape de structuration et de finition de ladite surface de glissement (21) dans des zones de ladite surface de glissement (21) définies à l'intérieur des cratères (22) et dans des zones de ladite surface de glissement (21) définies entre un cratère (22) et un autre, de manière à obtenir une pluralité de crêtes (24) de dimensions nanométriques et réparties sur la surface de glissement (21) de la base (11), dans lesdits cratères (22) et entre un cratère (22) et un autre.

2. Procédé selon la revendication 1, **caractérisé en ce qu'**à la fin de ladite première étape de coupe, lesdits cratères (22) sont répartis selon un motif (23) de préférence régulier sur la surface de glissement (21) de la base (11).

3. Procédé selon l'une quelconque des revendications ci-dessus, **caractérisé en ce que** ladite première étape de coupe est réalisée en utilisant un laser pulsé.

4. Procédé selon l'une quelconque des revendications ci-dessus, **caractérisé en ce que** lesdits cratères (22) ont une profondeur (P) variable entre environ 0,5 µm et environ 50 µm.

5. Procédé selon l'une quelconque des revendications ci-dessus, **caractérisé en ce que** lesdits cratères (22) ont un diamètre (D) variable entre environ 5 µm et environ 100 µm, et de préférence inférieur à 50 µm.

6. Procédé selon l'une quelconque des revendications ci-dessus, **caractérisé en ce que** ledit procédé de finition et de structuration sur la surface de glissement (21) est un procédé de nanostructuration réalisé par un procédé d'érosion ionique sur la surface de glissement (21).

7. Base de glissement comprenant au moins une surface de glissement (21), dans laquelle ladite surface de glissement (21) comprend une pluralité de cratères (22) ayant des dimensions micrométriques et ayant une profondeur (P) et un diamètre (D) contrôlés et une pluralité de crêtes (24) ayant des dimensions nanométriques et réparties dans des zones de la surface de glissement (21) de la base (11) situées dans lesdits cratères (22) et dans des zones situées entre un cratère (22) et un autre.

8. Base selon la revendication 7, **caractérisée en ce que** ladite base (11) est constituée par au moins une couche de matériau métallique ou d'alliages métalliques.

9. Base selon la revendication 7 ou la revendication 8, **caractérisée en ce que** ladite base (11) a une épaisseur variable entre environ 0,2 mm et environ 0,8 mm.

10. Dispositif de glissement comprenant une pluralité de couches (12-19) en chevauchement et au moins une base (11) munie d'au moins une surface de glissement (21), dans lequel ladite surface de glissement (21) comprend une pluralité de cratères (22) ayant des dimensions micrométriques et ayant une profondeur (P) et un diamètre (D) contrôlés et une pluralité de crêtes (24) ayant des dimensions nanométriques et réparties dans des zones de la surface de glissement (21) de la base (11) à l'intérieur desdits cratères (22) et dans des zones situées entre un cratère (22) et un autre.

11. Dispositif de glissement selon la revendication 10, **caractérisé en ce qu'**il comporte des bords réalisés d'une seule pièce avec la base (11).
